# EUROPEAN PATENT SPECIFICATION

(11) **EP 0 327 556 B1**
(45) Date of publication and mention of the grant of the patent: **04.03.1992**
(21) Application number: 87906835.1
(22) Date of filing: 19.10.1987
(51) Int. Cl.: C22C 21/00

(54) **RAPID SOLIDIFICATION ROUTE ALUMINIUM ALLOYS CONTAINING LITHIUM**
LITHIUM ENTHALTENDE ALUMINIUMLEGIERUNGEN, HERGESTELLT AUF DEM WEG DER RASCHEN ABKÜHLUNG
ALLIAGES A BASE D'ALUMINIUM CONTENANT DU LITHIUM OBTENUS PAR VOIE DE SOLIDIFICATION RAPIDE

(30) Priority: 21.10.1986 GB 8625189
(43) Date of publication of application: 16.08.1989
(73) Proprietor: Secretary of State for Defence in Her Britannic Majesty's Gov. of the United Kingdom of Great Britain and Northern Ireland, London SW1A 2HB (GB)
(72) Inventor: JONES, Edward, Sheffield SIB 5YW (GB); TSAKIROPOULOS, Panayiotis, Petersfield Hampshire (GB); PRATT, Charles, Robert, West Glamorgan (GB); GARDINER, Robert, William, Parnham, Surrey (GB); RESTALL, James, Edward, Surrey GU15 1DN (GB)
(74) Representative: Beckham, Robert William
(86) International application number: GB8700734
(87) International publication number: WO8803178

(56) References cited:
- CH-A- 0 216 204
- FR-A- 2 538 412
- Chemical Abstracts, vol. 100, no. 24, 11 June 1984, (Columbus, Ohio, US), E.S. Balmuth: "Particle size determination in an AL-3 Li alloy using DSC", see page 272, abstract 196289b, & Scr. Metall. 1984, 18(4), 301-4
- 4th International Aluminium Lithium Conference, ed. Les Editions de Physique, colloque C3, supplement no. 9, volume 48, septembre 1987, R.C.A. Pratt et al.: "Effect of dispersoid-forming additions on the response to heat treatment of splat-quenched Al-Li-X alloys", pages 341-346 ; see page 343, conclusions and page 345, table 2
- Metals & Materials, (Jan. 1987), page 15-20

## Description

This invention relates to aluminium based alloys containing lithium, made by the rapid solidification rate (RSR) route.

It is well known that lithium can be included in an aluminium alloy to reduce its density and increase its modulus of elasticity. Much work has been performed in this area on materials made by RSR routes as well as the more conventional wrought ingot route. RSR routes to the production of high modulus low density alloys based on aluminium-lithium offer at least the three following potential attractions:-
(1) a more uniform and refined microstructure including elimination of ingot-derived coarse metallic second phases that can act as sites for crack initiation and corrosion:
(11) incorporation of dispersoid phases that are more effective in homogenising slip than are phases incorporated via the ingot route, so improving ductility and toughness;
   and;
(111) incorporation of higher lithium contents than can be accommodated by the wrought ingot route (by avoidance of segregation limitations) thereby offering the prospect of more significant reductions in density and increases in modulus and strength.

This invention concerns especially the dispersoid phase aspect of the RSR route aluminium-lithium art. Several dispersoid-forming additions have been investigated previously. One prior art investigation looked at the effects of 0.2 to 0.6 weight percent additions of manganese, chromium, iron, cobalt, titanium and zirconium on an aluminium - 3 weight percent lithium alloy. Other additions which we know to have been investigated previously (in a variety of documents) are as follows (all proportions in weight percent): 1 to 7 silicon; 0.2 titanium; 0.4 chromium; 0.2 to 3 manganese; 0.5 iron; 0.2 to 1 cobalt; 0.04 yttrium, and 0.2 to 1 zirconium.

It is also known from FR-A-2 538 412 to produce rapidly solidified Al-Li-W alloys comprising 1-3% Li. and 0.05-0.3% W in proportions by weight and which may additionally contain 0.05-5.0% Cu and/or 0.5-8.0% Mg. The document states that such alloys are obtained with increased electrical resistivity compared to corresponding alloys formed by conventional ingot metallurgy.

The problem is one of developing a RSR route aluminium-lithium alloy having a good balance of those properties desirable especially for aerospace structural application, such desirable properties including strength, high modulus, ductility and fracture toughness together with low density; and the present invention tackles this problem by providing new additives for such alloys, that resist coarsening in the aluminium-base matrix at elevated temperatures of the level that is likely to be experienced in solution treatment, in artificial ageing or in service.

The invention comprises an alloy formed by a rapid solidification rate process comprising the following ingredients in proportions by weight:
Li 1 - 5%
one or more of the following refractory elements within the individual proportions stated below and in total proportion not exceeding 5% when present in combination
Nb 0.2 - 5.3%
Mo 0.2 - 5.0%
Hf 0.2 - 5.0%
Ta 0.2 - 5.0%
W 1.0 - 5.0%
with Al as balance save for incidental impurities and save for 5% in total of one or more of the following conventional strengthening ingredients within the individual proportions stated:
Cu 0 - 5%
Mg 0 - 5%
Zn 0 - 5%

If lithium is present in much greater proportion it would be likely to render the alloy overly brittle.

It has been found that the inclusion of such a refractory metal element in an aluminium-lithium base alloy confers improved strength to same (as reflected in the microhardness of RSR splats) and improved thermal stability (as reflected in the change of microhardness with exposure to temperatures representative of solution treatment temperature and artificial ageing temperatures). It is believed that these improved properties are consequent partly upon dispersoids formed within the aluminium matrix by the refractory metal element. It is expected that this benefit will not be significantly diminished by the presence in the base alloy of those ingredients other than lithium which have been added to aluminium-lithium alloys for strengthening purposes etc. A dispersion of the aluminium-refractory metal element compounds act to inhibit grain growth and thus help to retain the fine grain size inherent in RSR alloys. This fine grain size is important for the development of high strength and ductility. Solution heat treatment, quenching and ageing of the alloy results in the precipitation of aluminium-lithium based compounds as it would for dispersoid-free aluminium-lithium alloys. The presence of other elements such as copper, zinc and magnesium in an aluminium-lithium alloy which promote precipitation hardening in a solution treated alloy, is unlikely to markedly affect the grain growth inhibiting properties of the aluminium-refractory metal element dispersoid.

Various RSR methods well established in the art are suitable for the practice of the invention. RSR methods possess in common the imposition of a high cooling rate on an alloy from the liquid. RSR methods such as melt spraying, chill methods and weld methods are described in some depth in Rapid Solidification of Metals and Alloys by H Jones (published as Monograph No 8 by The Institution of Metallurgists) and in many other texts. The various RS routes differ from one another in their abilities in regard to control of cooling rate. The degree fo dispersoid refinement and the extension of solid solubility are dependent on the rate of cooling from the melt.

Much of the laboratory work in connection with the current invention has been performed using a twin piston splat quenching method as described at pages 11 and 12 of the aforementioned text by H Jones. This technique is not susceptible to scale up to an industrial scale. For such larger scale use alternative well established RSR methods such as gas atomising or planar flow casting would be suitable

The alloy may contain an ingredient or ingredients other than aluminium, lithium, and X such as those common in aluminium-lithium alloys, eg copper magnesium or zinc.

The alloy is exemplified by reference to the specific compositions given in Tables 1 2 and 3 are for the alloys when produced as RSR splats within an argon atmosphere by the twin piston technique. The splats produced were typically around 50um thick and the cooling rate developed by the RSR process was of the order of 10⁵ to 10⁶degrees Celcius per second. The recorded compositions shown in the first column of Tables 1 and 2 represent the measured composition of the source ingot. This will correspond closely to the composition of the splat at all times in the tests documented save in respect of the lithium content. The measured lithium content for most of the splats is given in parenthesis adjacent the relevent microhardness entry.

Table 1 below gives measurements fo microhardness (expressed in kg/mm²) as a function of time of exposure at 540 degrees Celcius this being a temperature representative of a solution treatment regime. The specimens were encapsulated prior to exposure within a quartz enclosure filled with argon. At completion of the exposure period the specimens were removed from the encapsulation and water-quenched to room temperature. Tantalum containing alloys are not documented in the quoted figures but are expected to have comparable properties.

Table 2 below documents variations in microhardness and lithium content for a test similar to that in Table 1 save that it was conducted at a temperature of 160 degrees Celcius which is a temperature representative fo artificial ageing conditions. Some of the specimens (those indicated) were subjected to a solution treatment fo 1 hour at 540 degrees Celcius followed by water-quenching to room temperature prior to ageing. The remainder were subjected to the ageing treatment from the 'as-splatted' condition.

It is recognised that the experimental results presented above document the properties of the claimed alloy only by reference to microhardness measurements of splat speciments. It is expected that these figures will to a large extent be a valid indication fo the strength and stability properties of the claimed alloy when produced on an industrial scale under suitable RSR condition.

Table 3 below documents one comparative test of an alloy of the invention against a reference alloy. The aluminium - 4 lithium - 0.6 molybdenum alloy was produced as RSR powder by inert gas atomising. The powder was canned and then extruded (without the usual intermediate degassing treatment) to round bar at a 25:1 reduction ratio. The extruded bar was solution treated at 540 degrees Celcius for one hour, water quenched, then aged for one hour at 160 degrees Celcius. The comparitive data relates to a comparable prior art alloy and the figures given are taken from a published work - a paper by P J Meschter et al at page 85 et seq of Aluminium-Lithium III (the proceedings of the Third International Aluminium-Lithium Conference) published by The Institute of Metals. The data given is for a alloy of aluminium - 4 lithium - 0.2 zirconium extruded from RSR powder, solution treated at 588 degrees Celcius then aged for one hour at 160 degrees Celcius.

The above quoted alloy of the invention is unlikely to be representative of the true merits of the invention for the figures document a process not optimised with regard to the RSR powder production and without the important degassing stage. However the quoted alloy, even in this condition, shows a useful increase in strength over the reference alloy. It should be recognised that although this comparison is fair with regard to the equivalence of the materials documented it does not document the best of prior art materials nor is it likely to document the best materials of the invention.

As mentioned previously the alloy of the invention is not limited to an aluminium - lithium - X system for it is possible that additions other than lithium and X will be incorporated within the aluminium base in order to yield a material having a better blend of properties than can be secured through a ternary alloy. It is postulated that the alloy could include up to 5 percent or thereabouts of one or more ingredients selected from the group consisting of copper zinc and magnesium.

## Claims

1. An alloy formed by a rapid solidification rate process comprising the following ingredients in proportions by weight:
Li 1-5%
one or more of the following refractory elements within the individual proportions stated below and in total proportion not exceeding 52 when present in combination
Nb 0.2 - 5.3%
Mo 0.2 - 5.0%
Hf 0.2 - 5.0%
Ta 0.2 - 5.0%
W 1.0 - 5.0%
with Al as balance save for incidental impurities and save for up to 5% in total of one or more of the following conventional strengthening ingredients within the individual proportions stated:
Cu 0-5%
Mg 0-5%
Zn 0-5%

2. An alloy as claimed in claim 1 comprising 1 to 5 percent of lithium and 1 to 5 percent of niobium, in proportions by weight.

3. An alloy as claimed in claim 1 comprising 1 to 5 percent of lithium and 0.5 to 1.5 percent of molybdenum, in proportions by weight.

4. An alloy as claimed in claim 1 comprising 1 to 5 percent of lithium and 3 to 5 percent of hafnium, in proportions by weight.

5. An alloy as claimed in claim 1 comprising 1 to 5 percent of lithium and 1 to 3 percent of tungsten, in proportions by weight.

## Patentansprüche

1. Durch Schnellerstarrung gebildete Legierung aus den nachstehenden Bestandteilen, jeweils in Gewichtsprozent:
Li 1-5%
einem oder mehreren der nachstehenden feuerfesten Elemente innerhalb der nachstehend angegebenen Einzelanteile und zusammen in einem 5% nicht übersteigenden Gesamtanteil;
Nb 0,2 - 5,3%
Mo 0,2 - 5,0%
Hf 0,2 - 5,0%
Ta 0,2 - 5,0%
W 1,0 - 5,0%
Rest Al, außer zufälligen Verunreinigungen sowie bis zu 5% insgesamt einer oder mehrere der nachstehenden üblichen verstärkenden Bestandteile innerhalb der angegebenen Einzelanteile:
Cu 0-5%
Mg 0-5%
Zn 0-5%

2. Legierung nach Anspruch 1 mit 1 bis 5 Gew.-% Lithium und 1 bis 5 Gew.-% Niob,

3. Legierung nach Anspruch 1 mit 1 bis 5 Gew.-% Lithium und 0,5 bis 1,5 Gew.y% Molybdän.

4. Legierung nach Anspruch 1 mit 1 bis 5 Gew.-% Lithium und 3 bis 5 Gew.m% Hafnium.

5. Legierung nach Anspruch 1 mit 1 bis 5 Gew. -% Lithium und 1 bis 3 Gew. -% Wolfram.

## Revendications

1. Alliage formé par un procédé de solidification rapide, comprenant les constituants suivants en les proportions pondérales suivantes :
Li 1 - 5%
un ou plusieurs des éléments réfractaires suivants, en les proportions individuelles ci-après et en proportion totale n'excédent pas 5% lorsqu'ils sont présents en combinaison
Nb 0,2 - 5,3%
Mo 0,2 - 5,0%
Hf 0,2 - 5,0%
Ta 0,2 - 5,0%
W 1,0 - 5,0%
et Al pour le reste, sauf les impuretés accidentelles et sauf jusqu'à 5% au total d'un ou plusieurs des constituants augmentant la résistance classiques suivants en les proportions individuelles indiquées :
Cu 0 - 5%
Mg 0 - 5%
Zn 0 - 5%

2. Alliage suivant la revendication 1, comprenant 1 à 5% de lithium et 1 à 5% de niobium, en proportions pondérales.

3. Alliage suivant la revendication 1, comprenant 1à 5% de lithium et 0,5 à 1,5% de molybdène, en proportions pondérales.

4. Alliage suivant la revendication 1, comprenant 1 à 5% de lithium et 3 à 5% de hafnium, en proportions pondérales.

5. Alliage suivant la revendication 1, comprenant 1 à 5% de lithium et 1 à 3% de tungstène, en proportions pondérales.
